

Patented May 20, 1952

2,597,412

# UNITED STATES PATENT OFFICE

2,597,412

## DIAZOTYPE COMPOSITIONS CONTAINING UNSATURATED ALKYL N-DERIVATIVES OF AMINO DIAZOS

William H. von Glahn, Loudonville, and Lester N. Stanley, Delmar, N. Y., assignors to General Aniline & Film Corporation, New York, N. Y., a corporation of Delaware

No Drawing. Application December 29, 1948,  
Serial No. 68,072

5 Claims. (Cl. 95—7)

1

This invention relates to the production of diazotype light sensitive layers or diazotype materials and more particularly to diazotype materials wherein the light sensitive agent is a diazo derivative of an aromatic p-diamine.

The diazotype process, as is well known, involves the treating of a carrier or base, usually paper which may be either opaque or transparentized, or film of the cellulose ester or cellulose ether type, with a sensitizing composition containing a diazo compound as the light sensitive element. This treated base is exposed to actinic light through a pattern and a positive reproduction of the original obtained by development of the undecomposed diazo compound under the protected portions of the pattern, by means of alkaline coupling with an azo dye coupling component. The azo dye coupling component used for development of the image may be contained in an alkaline developing solution, as is the case in the so-called wet development or one-component process. In the dry development or two-component diazotype process, the sensitizing composition with which the base material is treated contains both the diazo compound and the azo coupling component. Here, the azo dye image is formed after exposure of the sensitized material by subjecting the exposed material to the action of alkaline vapors such as ammonia vapors. The diazotype photosensitive material for the two-component process must have good stability against precoupling, so that the sensitized layers may be stored for reasonable periods of time under average conditions of temperature and humidity prior to use.

The two-component diazotype process is extensively used for the preparation of intermediate or transition prints in cases where it is desired to make a large number of reproductions. By making such an intermediate diazotype transition print it is only necessary to expose the original once or a few times since the transition print is thereafter used to make the desired number of duplicates. Consequently, a valuable original drawing may be spared the rigorous treatment of repeated exposures which might result in the impairment of even destruction of the original drawing. In producing an intermediate diazotype print, a transparent or semi-transparent paper or film is coated with a light sensitive diazotype sensitizing solution and dried. It is then exposed to actinic light rays, particularly from a source rich in the ultraviolet band of from 3600 Å. to 4200 Å. under the drawing or picture to be reproduced. The image is then developed by contacting the exposed light sensitive surface, if it be a two-component diazotype, to ammonia vapors.

The efficiency of transition prints depends upon the covering power or photographic density of the azo dye image produced and particularly

2

its opacity to ultraviolet light, and also upon the transparency of the background surrounding the developed pattern. The clarity of the background, and hence its transparency, is decreased if color has been produced therein due to the residual or undecomposed diazo compound, or to premature coupling of the dye components prior to use. Such casual color in the background of the intermediate print will be reproduced in subsequent copies due to the ultraviolet absorbing qualities of the transition color.

The efficiency of transition prints also to some extent depends upon the depth or visual density of the image produced. Light colored images of poor visual density which may satisfy the requirements of opacity to ultraviolet light and ability to resist precoupling nevertheless have the disadvantage of rendering difficult the detection of flaws in the intermediate image, and it is often necessary to make a test print from the transition print of a deep contrast before such flaws can be detected, with consequent loss of time, convenience and economy.

We have now found that a new class of diazo compounds which are derived by mono diazotization of a p-phenylene diamine containing at least one unsaturated lower alkyl substituent on the undiazotized amino group give excellent results when used as the light sensitive agents of a diazotype layer. This new class of diazo compounds may be used with coupling components which will produce dye images in dark shades such as blues or those which will produce ultraviolet light absorbing shades such as sepia for use in diazotype transition printing. The amines from which the diazo compounds of this class are derived have the formula



wherein R<sub>1</sub> is an alkyl group of less than five carbon atoms containing at least one unsaturated carbon to carbon linkage and such radicals containing a hydroxyl group and R<sub>2</sub> is hydrogen, alkyl, hydroxy alkyl, aryl, cycloaliphatic or another R<sub>1</sub> radical. Examples of diazo compounds of this class include:

- 55 N-allylamino-p-benzene diazonium chloride  
N-methallylamino-p-benzene diazonium chloride  
N-methyl-N-(2-hydroxy-3-butenyl)amino-p-benzene diazonium chloride  
60 N-hydroxyethyl-N-(2-hydroxy-3-butenyl)amino-p-benzene diazonium chloride

N-phenyl-N-allylamino- p -benzene diazonium chloride  
 N,N-di(2-hydroxy-3-butenyl) -amino- p -benzene diazonium chloride  
 N-cyclohexyl - N(2-hydroxy- 3 -butenyl) amino- p -benzene diazonium chloride  
 N-methyl-N-butadienyl-amino - p - benzene diazonium chloride

It has been found that diazo compounds of this class when employed with one of the azo components generally used for diazotype work either by the dry development process wherein the diazo compound and coupling component are both contained in the light sensitive layer or by the wet development process wherein only the diazo compound is contained in the light sensitive layer and the azo component is applied as part of an alkaline developing solution, reproductions can be obtained having images of bright dark tones on a clear white background wherein the images are wash-fast, light-fast, permanent and have good properties of photographic definition. These diazo compounds also possess good stability in the unexposed stage when both the diazo and the azo coupling component are incorporated in a two-component system for the dry developing diazotype process. By reason of the fact that they decompose completely and readily upon exposure to light, particularly the actinic rays of ultraviolet light, the diazo compounds of this class are characterized by an excellent printing speed when used either in a two-component or one-component diazotype system. When used in conjunction with the proper azo components such as resorcinol and resorcinol derivatives these diazos will produce the image in a sepia shade which has excellent photographic density or opacity to ultraviolet light. These sepia reproductions having a very high degree of opacity will yield clear and sharply defined copies in the final print when applied to diazotype transition printing. The intermediate sepia reproductions will not blur or offset when the print is used as a mask.

The diazo compounds of this class may be prepared by one of several methods. They may be prepared by reacting unsaturated alkyl halides, such allyliodide and methallyliodide with aromatic amines such as aniline, N-methylaniline, o-toluidine, N-hydroxyethyl-o-toluidine and the like. The reaction product of the alkyl halide and the aromatic amine is then nitrosated, reduced, diazotized and stabilized in the usual manner. In order to prepare those derivatives which contain a hydroxy group in addition to an unsaturated group in the N-substituent or substituents, the aryl amines are reacted with an unsaturated alkylene oxide, such as 3,4-epoxy-1-butene. The reaction product is then nitrosated, reduced, diazotized and stabilized in the same manner as above.

The diazotype layers produced from this class of diazo compounds may be effected in the usual manner, wherein the base or support carrying or containing the light sensitive compounds, the azo components and other coating materials is coated, dipped, brushed or sprayed with the sensitizing solution, the particular type of application generally depending upon the character of the carrier employed. As carriers, such materials as paper or cloth which may be opaque, semi-transparent or of a transparentized type; film such as prepared from cellulose nitrate, cellulose acetate, or cellulose esters, regenerated cellulose, superpolymers and polymerization

products; ceramic plates or sheet metal may be employed. Where paper is used as the base or support for the light sensitive coating, the coated solution is generally applied by using a trough and doctor blade but may, if desired, be brushed or sprayed. When a film or spirit soluble plastic is used as a support swelling agents should be added to the coating solution in order to obtain proper penetration and the solution is generally applied by a dipping method.

In addition to the diazo compound, azo component and such swelling agents as may be added, the coated solution may contain the usual adjuncts such as metal salts designed to intensify the dye image and increase its water resistance, such as aluminum sulfate, titanium ammonium fluoride and nickel sulfate; stabilizing agents such as thiourea, thiosinamine and naphthalenetrisulfonic acid; acids designed to retard precoupling, such as citric acid, tartaric acid and boric acid; and hygroscopic agents such as glycol, glycerine and dextrin to protect the light sensitive layer from excess moisture.

When single component diazotype layers are desired the coating methods for producing the light sensitive layer on the desired support are the same as employed for the production of two-component diazotype layers except that the azo component is omitted from the coating solution as previously pointed out and as is well known in the art. The azo component is then added to the alkaline developing solution. As will be obvious adjuncts added to the coating solution to improve its precoupling properties will be unnecessary in the case of one-component solutions.

As coupling components for either the one-component or two-component diazotype systems we may use any azo coupling component known to be suitable for diazotype light sensitive layers. As examples of these there may be mentioned:

- (1) 2,3-dihydroxy naphthalene and its sulfonic acid derivatives
- (2) Phloroglucin
- (3) Naphthalene guanidines, such as—  
 7-hydroxy naphthalene-1-guanidine  
 5-hydroxy naphthalene-1-biguaniidine
- (4) Acetoacetic acid amides, such as—  
 N-(cyclohexyl) acetoacetamide  
 N-(benzyl) acetoacetamide  
 N-( $\alpha$ -pyridyl) acetoacetamide
- (5) Substituted naphthols, such as—2,6-dimethyl-8-hydroxy naphthalene and its reaction product with formaldehyde-dimethylamine
- (6) Hydroxynaphtho-imidazoles, such as—  
 7-hydroxynaphtho-1',2':4,5 imidazole  
 2-carbethoxy - 7' - hydroxynaphtho-1',-2':4,5-imidazole
- (7) Phenol and phenol derivatives
- (8) Cresols
- (9) Resorcinol and resorcinol derivatives, such as—  
 4-chlororesorcinol  
 Dichlororesorcinol  
 Resorcinol esters and ethers

Some of these azo components, notably those of the resorcinol family which will produce sepia images have a fast coupling rate. This tends to impair the precoupling stability of a two-component system containing such an azo component. Since it is desirable to use these azo components which will produce sepia shades in the production of diazotype transparencies, precoupling in-

stability is a decided disadvantage as background color will be produced as a result of such instability and this background color will absorb actinic light in areas where the transparencies should transmit light. Although some of the azo coupling components which produce sepia images are more stable than others this disadvantage which is inherent in the class of azo components which produce the ultraviolet absorbing shades is modified or overcome when using the diazo compounds of this invention.

The following examples will serve to illustrate further the preparation of diazotype photo-printing materials from the diazo compounds of our invention and it being understood that the invention is not limited to the particular materials or preparations therein described. Unless otherwise specified, the parts are by weight.

#### EXAMPLE 1

Transparentized paper is coated with a coating solution containing the following materials per 100 parts of water:

3.2 parts N - allylamino - p - benzene diazonium chloride CdCl<sub>2</sub> double salt  
1.8 parts resorcinol  
8.0 parts citric acid  
4.0 parts thiourea

The thus coated transparentized paper is then dried and exposed to light under a pattern and the print developed by drying the exposed diazotype coated paper through ammonia fumes. The sepia colored positive reproduction is obtained on a clear background. The opacity to ultraviolet light of the developed image is outstanding. Visual appearance, wash and light-fastness and fastness to offset are also good. This sepia dye reproduction may, therefore, be used as a positive original with ordinary diazotype reproduction media or other light sensitive reproduction media to yield excellent reproductions in any desired color. Its printing speed during exposure is excellent and its resistance to precoupling prior to exposure is also very satisfactory.

#### EXAMPLE 2

Transparentized paper is coated with a solution containing the following materials per 100 parts of water:

3.5 parts N-methyl-N-methallylamino-p-benzene diazonium chloride-ZnCl<sub>2</sub> double salt  
2.7 parts 4,6-dichlororesorcinol  
8.0 parts citric acid  
4.0 parts thiourea  
3.0 parts isopropanol

The thus coated paper is dried in the usual manner. It has excellent precoupling stability and can be stored for long periods of time without any noticeable spontaneous formation of color due to coupling of the dye components. When exposed to the actinic rays of ultraviolet light under a positive original and developed with ammonia vapor this coated transparency produces a well defined sepia colored positive reproduction of the original on a clear background. The opacity of the sepia colored image and its ability to thus absorb ultraviolet rays in the colored areas so as to prevent printing through in those areas is outstanding. The visual appearance, wash and light fastness and fastness to offset of the sepia colored image are also good. As in Example 1, the product of this example may be used in transition printing thus, the sepia colored image derived from the positive original by

exposure and development may be employed in place of the original for printing through on the ordinary diazotype reproduction media or other photo-printing reproduction media for the purpose of producing additional reproductions of any desired color.

#### EXAMPLE 3

Transparentized paper is coated with a solution containing the following materials per 100 parts of water:

3.6 parts N-methyl-N-(2-hydroxy-3-but enyl)-amino-p-benzene diazonium chloride ZnCl<sub>2</sub> double salt  
15 2.5 parts 4-bromoresorcinol  
8.0 parts citric acid  
4.0 parts thiourea  
5.0 parts isopropanol

The thus coated paper is dried in the usual manner and is found to have excellent stability against precoupling during storage and when exposed to ultraviolet light under a positive original and developed with ammonia vapor it produces a well defined sepia colored image which is a positive reproduction of the original on a clear background. The opacity of this image to ultraviolet light is outstanding. Its visual appearance, wash and light fastness and fastness to offset are also good. This sepia dye reproduction image may, therefore, be used in place of the positive original for the production of further copies by printing through on to ordinary diazotype reproduction media or other photo-printing media to yield excellent reproductions in any desired color.

#### EXAMPLE 4

Diazotype paper stock is coated with a solution containing the following material per 100 parts of water:

40 2.4 parts N-hydroxyethyl-N-(2-hydroxy-3-but enyl)-amino-p-benzene diazonium chloride-ZnCl<sub>2</sub> double salt  
1.5 parts 2,3-dihydroxynaphthalene-6-sulfonic acid  
45 8.0 parts citric acid  
4.0 parts thiourea  
5.0 parts isopropanol

The thus coated paper is dried in the usual manner and is found to have excellent precoupling stability. When exposed to the actinic rays of ultraviolet light under a pattern and developed with ammonia vapor it gives a positive reproduction of the original in an attractive blue shade against a clear white background having no discernible discoloration due to premature coupling of the dye components.

#### EXAMPLE 5

60 Transparentized paper is coated with a coating solution containing the following material per 100 parts of water:

3.6 parts N-phenyl-N-allylamino-p-benzene diazonium chloride ZnCl<sub>2</sub> double salt  
65 2.6 parts resorcinol-4-sulfonic acid  
8.0 parts citric acid  
4.0 parts thiourea  
5.0 cc. isopropanol

70 The thus coated transparency is dried in the usual manner and is found to have excellent precoupling stability. When exposed to ultraviolet light under a positive original and developed with ammonia vapor a sepia colored positive reproduction of the original on a clear background is ob-

tained. The opacity of the sepia image or its ability to absorb ultraviolet light emanations is outstanding. Its visual appearance, wash and light fastness and fastness to offset are also good. This sepia dye reproduction image may be used as a positive original with ordinary diazotype reproduction media or other photo-printing media to yield excellent reproductions in any desired color.

#### EXAMPLE 6

Transparentized paper is coated with a coating solution containing the following material per 100 parts of water:

3.6 parts N,N-di(2-hydroxy-3-butenyl)-amino-p-benzene diazonium chloride-ZnCl<sub>2</sub> double salt  
 1.8 parts resorcinol  
 8.0 parts citric acid  
 4.0 parts thiourea  
 5.0 cc. isopropanol

The thus coated transparency is dried in the usual manner. It is found to have excellent pre-coupling stability and when exposed to the actinic rays of ultraviolet light under a positive original and developed with ammonia vapor a sepia colored positive reproduction of the original on a clear background is obtained. The opacity of the image or its ability to absorb ultraviolet light emanations is outstanding. Its visual appear-

ance, wash and light fastness and fastness to offset are also good. In view of the excellent pre-coupling stability of the unexposed light sensitive coating and the outstanding opacity of the image produced by exposure and development, this product is eminently suited for diazotype transition printing and when used as an intermediate positive original it will produce excellent reproductions on ordinary diazotype reproduction media or other photoprinting media in any desired color.

Upon substituting N<sup>1</sup>-methyl-N-butadienyl-amino-p-benzene diazonium chloride-ZnCl<sub>2</sub> double salt for the diazo compound of this example light sensitive coatings having similar properties are obtained:

#### EXAMPLE 7

Transparentized paper is coated with a solution containing the following material per 100 parts of water:

3.5 parts N-cyclohexyl-N-(2-hydroxy-3-butene)-amino-p-benzene diazonium chloride-ZnCl<sub>2</sub> double salt  
 5 cc. isopropanol

The thus coated paper is dried in the usual manner. Upon exposing it under a pattern and developed in a mildly alkaline solution containing resorcinol excellent sepia colored prints on a clear background are obtained.

#### Tables of structural formulae

##### I. BASES FOR DIAZO DERIVATIVES

| Compound                                                 | Structural Formula |
|----------------------------------------------------------|--------------------|
| (1) p-N-allylaminobenzene                                |                    |
| (2) p-N-methyl-N-methallylaminobenzene                   |                    |
| (3) p-N-methyl-N-(2-hydroxy-3-butene)-aminoaniline       |                    |
| (4) p-N-hydroxyethyl-N-(2-hydroxy-3-butene)-aminoaniline |                    |
| (5) p-N-phenyl-N-allylaminobenzene                       |                    |
| (6) p-N,N-di(2-hydroxy-3-butene)-aminoaniline            |                    |
| (7) p-N-cyclohexyl-N-(2-hydroxy-3-butene)-aminoaniline   |                    |
| (8) p-N-methyl-N-butadienyl-aminobenzene                 |                    |

## II. DIAZONIUM SALTS

| Compound                                                                                                     | Structural Formula                                                                                                                                    |
|--------------------------------------------------------------------------------------------------------------|-------------------------------------------------------------------------------------------------------------------------------------------------------|
| (1) N-allylamino-p-benzene diazonium chloride CdCl <sub>2</sub> double salt                                  | <br>$\text{N}=\text{NCl} \text{ } \text{ } \text{ } \text{ZnCl}_2$   |
| (2) N-methyl-N-methallylamino-p-benzene diazonium chloride ZnCl <sub>2</sub> double salt                     | <br>$\text{N}=\text{NCl} \text{ } \text{ } \text{ } \text{ZnCl}_2$   |
| (3) N-methyl-N-(2-hydroxy-3-butenyl)-amino-p-benzene diazonium chloride ZnCl <sub>2</sub> double salt        | <br>$\text{N}=\text{NCl} \text{ } \text{ } \text{ } \text{ZnCl}_2$   |
| (4) N-hydroxyethyl-N-(2-hydroxy-3-but enyl)-amino-p-benzene diazonium chloride ZnCl <sub>2</sub> double salt | <br>$\text{N}=\text{NCl} \text{ } \text{ } \text{ } \text{ZnCl}_2$  |
| (5) N-phenyl-N-allylamino-p-benzene diazonium chloride ZnCl <sub>2</sub> double salt                         | <br>$\text{N}=\text{NCl} \text{ } \text{ } \text{ } \text{ZnCl}_2$ |
| (6) N,N-di(2-hydroxy-3-but enyl)-amino-p-benzene diazonium chloride ZnCl <sub>2</sub> double salt            | <br>$\text{N}=\text{NCl} \text{ } \text{ } \text{ } \text{ZnCl}_2$ |
| (7) N-cyclohexyl-N-(2-hydroxy-3-but enyl)-amino-p-benzene diazonium chloride ZnCl <sub>2</sub> double salt   | <br>$\text{N}=\text{NCl} \text{ } \text{ } \text{ } \text{ZnCl}_2$ |

## We claim:

1. Diazotype materials comprising a base having a photosensitive coating which includes a light sensitive mono diazo derivative of an aromatic p-diamine of the benzene series having the following formula



wherein R<sub>1</sub> is a member of the group consisting of alkyl radicals of less than five carbon atoms containing at least one unsaturated carbon to carbon linkage and such radicals containing a hydroxyl group and R<sub>2</sub> is a member of the group consisting of hydrogen, alkyl, hydroxyalkyl, aryl, cycloaliphatic and R<sub>1</sub> radicals.

2. Diazotype materials comprising a base having a photosensitive coating which includes a light sensitive mono diazo derivative of an aromatic p-diamine of the benzene series having the formula



wherein R<sub>1</sub> is a member of the group consisting of alkyl radicals of less than five carbon atoms containing at least one unsaturated carbon to carbon linkage and such radicals containing a hydroxyl group and R<sub>2</sub> is a member of the group consisting of hydrogen, alkyl, hydroxyalkyl, aryl, cycloaliphatic and R<sub>1</sub> radicals and an azo dye coupling component.

3. A diazotype material comprising a base having a photosensitive coating which includes a light sensitive mono diazo derivative of p-N-allylaminoaniline and an azo dye coupling component.

4. A diazotype material comprising a base having a photosensitive coating which includes a light sensitive mono diazo derivative of p-N-methyl-N-methallylamino aniline and an azo dye coupling component.

5. A diazotype material comprising a base having a photosensitive coating which includes a light sensitive mono diazo derivative of p-N-methyl-N-(2-hydroxy-3-but enyl)aminoaniline and an azo dye coupling component.

60 WILLIAM H. VON GLAHN.  
LESTER N. STANLEY.

## REFERENCES CITED

The following references are of record in the 65 file of this patent:

## UNITED STATES PATENTS

| Number       | Name              | Date         |
|--------------|-------------------|--------------|
| 1,870,930    | Sprongerts et al. | Aug. 9, 1932 |
| 70 2,397,927 | Dickey et al.     | Apr. 9, 1946 |